

1,325,890.

L. FREUDER.

LITHOGRAPHY.

APPLICATION FILED NOV. 26, 1913.

Patented Dec. 23, 1919.



Fig. 1.



Fig. 2.

WITNESSES:

F. G. Stallman  
Wm. J. E. Hen

INVENTOR

Leo Freuder  
BY  
Ashley & Lechner  
ATTORNEYS

# UNITED STATES PATENT OFFICE.

LEO FREUDER, OF BROOKLYN, NEW YORK.

## LITHOGRAPHY.

1,325,890.

Specification of Letters Patent. Patented Dec. 23, 1919.

Application filed November 26, 1913. Serial No. 803,122.

*To all whom it may concern:*

Be it known that I, LEO FREUDER, a citizen of the United States, and a resident of Brooklyn, in the county of Kings and State 5 of New York, have invented certain new and useful Improvements in Lithography, of which the following is a specification.

This invention relates to lithography.

According to the usual processes in lithography hitherto employed, a key plate has to be prepared by the lithographic artist by 10 carefully reproducing every line, shadow and tone of the original. This is accomplished generally by making a series of dots 15 with a pen, known as stipple work. Where the shadows are deep the dots are large and close together; at the intermediate tones the dots are smaller and farther apart. This is a very laborious and tedious operation requiring often a month or more to turn out 20 the plates for the press. In some classes of work the surface of the key plate or stone is roughened and a crayon is used instead of the pen. This also requires a lot of very 25 careful hand work and has the disadvantage of the difficulty with which impressions are taken from a stone so prepared. Thus, the key stone itself has to be used as the press stone. In smaller work this process is al- 30 most prohibitive as the cost of printing is too high unless a number of impressions are taken on the press stone so as to make a number of prints at each operation of the press.

35 With the advent of photolithography some of the hand work of the lithographic artist has been dispensed with but a great portion of hand work still remains, and, moreover, a disturbing element is introduced 40 in the form of the screened negative. The tints in the picture to be reproduced are broken up into a series of dots through the action of the screen and thus in places where the high lights are found there are dots to 45 be taken out and in the shadows there are portions to be filled in. All this has to be done on the key plate by the lithographic artist and to secure good results a high degree of skill is required. Moreover, the dots 50 in the half tones appear very mechanical and detract considerably from the artistic

effect as compared with the original to be reproduced. There can be no gradual gradation of tone as found in all high grade artistic work. The sensitizer used is asphaltum or bichromate. If the plate is a little over exposed or under exposed it is spoiled and must be thrown away and new plate printed. Moreover, these sensitizers are otherwise more or less uncertain in their 60 action.

The present invention has for its principal object to provide a process in which all hand work requiring a lithographic artist or finisher is dispensed with, the screen 65 is eliminated, the results are absolutely uniform and certain, while the quality of the work is superior to that produced by the best of lithographic artists. The different tones are produced through a grain 70 which is more open or close according to the tone values and the minutest graduation in tone is faithfully represented with the utmost accuracy. The cost of producing the printing plate is reduced very greatly and 75 the time which it takes to prepare the plates from the copy is a small fraction of the time it takes with the processes known hitherto.

The various further objects and advantages will appear more fully from the detailed description, and the features of novelty will be particularly pointed out in the claims.

In the accompanying drawing.

85 Figure 1 is a diagrammatic view illustrating on an enlarged scale the character of the grain produced.

Fig. 2 is a diagrammatic view illustrating the manner in which the impressions are 90 taken from the key plate upon the press plate.

### Preparation of the key plate.

The material which I use for my key plate 95 may be any of the materials now used such as stone, glass, zinc or aluminum and in fact, any other suitable flexible material such as linen or rubber. The plate is first coated with a substratum of a suitable adhesive substance such as sodium silicate dissolved in 100 ten parts of a solution having albumen in a

finely divided state. I find that beer from which carbonic acid gas has been extracted answers the purpose of this solution. The plate is then coated with a stock solution 5 which can be used for a number of plates. This stock solution is composed of,

1. A gelatinous or gummy organic substance such as glue, gelatin, dextrin, sugar, or the like.
- 10 2. A sensitizer, preferably potassium bichromate or ammonium bichromate.
3. An agent which expands upon absorption of moisture, preferably calcium chlorid.

This solution is sensitive to light only 15 when dry, otherwise it is not sensitive. It can therefore be kept in stock for considerable time without deteriorating. I have found that the best proportions for the coating are as follows:

- 20 Solution 1: 1 part of gelatin in 10 parts of water.

Solution 2: 1 part of bichromate and 1 part of calcium chlorid in 10 parts of water.

These solutions are kept separate and are 25 mixed only immediately before being used upon the plate. When the same are to be applied, I add 330 gm. of Solution 1, 90 gm. of

Solution 2, the mixture is stirred well, heated to a temperature below boiling point, 30 filtered and then the plate may be coated.

The latter is then placed in a heating oven, particularly constructed for the purpose, and dried. It is necessary that during the drying process, the plate be protected from 35 air currents, as a slight disturbance is liable to cause a ripple on the surface of the plate which may appear later on the work. The temperature to which the plate is subjected in the oven depends upon the fineness of the

40 grain desired in the work. In the usual run of work, the best grains may be obtained between temperatures of 50° and 60° C. At or below 50°, the grain is finer, at higher temperature the grain is coarser. The plates 45 so prepared can be stored and kept for twelve or fourteen days without deterioration in their actinic properties.

When the subject is to be reproduced, assuming that a suitable plate is had in stock, 50 the first step is to make a photographic negative or a number of negatives, if the subject is to be reproduced in colors, using the well known color filters. The negative is then put in a printing frame, the coated plate placed on top of the same and exposed 55 through the negative to light from three to fifteen minutes according to the strength of the source of light. When the plate has been sufficiently exposed, it is removed from 60 the frame and washed in water until all the bichromate is washed out, leaving an image of a brownish color upon the plate. If the plate is a little over or under exposed, it will do no harm as this may be compensated

for by the degree of inking in the further manipulation. After the bichromate is washed out, the printing quality of the plate is improved as follows: The plate is leveled and covered with a solution consisting of one part water, one part glycerin and a small 70 amount of sodium chlorid according to the humidity of the air and the quality of the gelatin used in the plate. To about 225 gm. of a solution of water and glycerin, I add, under ordinary conditions, about 2 gm. of 75 sodium chlorid. The plate is allowed to soak in this solution from 15 to 30 minutes or more according to the quality of the gelatin and the degree of exposure. The moisture is then taken off with a fine sponge and the plate is inserted in the same oven in which it was previously dried and subjected to a heat of 50° C. until the plate feels somewhat tacky, which occurs usually within two to five minutes. The heat is then turned off, 80 the plate is cooled and the same is ready for making off-sets upon the press plate.

When the key plate is inked with the usual lithographic ink and a proof taken, it is found that the surface is broken up into a 90 grain formed by sinuous interwoven somewhat broken lines having a flaky appearance. Referring to Fig. 1 the upper square shows on an enlarged scale the character in the darker and intermediate tones and in the 95 lower square the lighter tones and the high lights. It will be noted that a series of sinuous lines 10 are formed from which radiate needles or tendrils 11. The general size of the grain depends upon the degree of heat 100 to which the plate has been subjected while the grain, itself is produced by the expansion of the calcium chlorid in absorbing water. At the portions of the plate which have seen a lesser amount of light, the gelatin is comparatively soft and permits the moisture to percolate therethrough and be absorbed by the calcium chlorid. The latter in absorbing the water expands and thus breaks up the hardened gelatin into the 105 grain described. Where the plate has seen more light corresponding to the shadows of the subject, the gelatin has become so hardened that less water will be absorbed and will also to a greater degree resist the force 110 tending to break it up; thus the grain is close, consequently printing darker. Where the plate has seen most light, corresponding to the deep shadows of the subject the gelatin may become so hardened as to prevent 115 the absorption of practically any water by the calcium chlorid or if some small amount is absorbed the gelatin is too tough to be broken up. Thus the plate prints solid black at the deep shadows, as it should. Where 120 the plate has seen no light whatever corresponding to the high lights of the subject, the gelatin is entirely soft, thus permitting 125

a very large amount of water to be absorbed preventing the gelatin from taking up any ink and leaving the print entirely white. The intermediate tones vary proportionately 5 in the degree of the openness of the grain, thus faithfully reproducing with great accuracy every tone variation of the subject.

*Preparation of the press plate.*

10 The press plate is preferably prepared from the key plate in an offset press as follows: Referring to Fig. 2, the key plate 20 is placed on the bed 21 of the offset press and the press plate 22 is placed upon the bed 23. 15 The offset roller 24 which is provided with a toothed wheel 25 engaging with a rack 26 formed upon the bed is located between two plates and may take the offset from the key plate and print the same upon the press 20 plate. Any suitable material may be used for the press plate, such as aluminum or zinc or stone. When the press plate has received the impression, the same is examined carefully and parts which have not the desired 25 strength are left open for correction and the rest of the plate is covered with gum arabic or gamboge for protection against the next impression. The key plate is then rolled up again with ink and an impression 30 is again taken on the press plate. The part which has been left open is thus strengthened and when the gum arabic is washed off from the rest of the plate, the corrected part has the desired strength compared with the 35 other parts of the plate. If desired, corrections may be made directly on the key plate with the aid of an air brush using steam instead of air. The portions to be weakened or reduced are subjected to the current of 40 steam, the gelatin absorbing more moisture and thus subsequently taking less ink. Also if it is desired to strengthen or increase any portion of the plate, the rest of the plate may be subjected to the current of steam 45 from the air brush and thus the part not so subjected will be relatively stronger or increased. This strengthening may also be accomplished by subjecting the particular part to be strengthened to a current of air from 50 the air brush containing some suitable hardening agent which acts upon the gelatin. If desired, the usual transfer paper method which has heretofore been employed to transfer the impression from the key stone 55 to the press stone can be entirely eliminated and the impressions of the key stone may be multiplied upon the press stone by shifting the former upon the bed of the press. In this method of manipulation, assurance may 60 be had that the various impressions upon the press plate are of equal strength, as the proof may be kept at hand with which the impressions are compared. If an impression is too light, another offset may be taken

from the key plate and printed over the previous impression. 65

*Etching of the press plate.*

After the impression is taken upon the press plate, the same may be etched in some 70 suitable manner:

In the preparation of the key plate, I have described the sensitizer as being applied to the plate in the form of a solution together with the printing medium. In 75 some cases, however, I may with advantage apply the sensitizer in the form of a dust upon the printing medium which is otherwise prepared as above described. In such case, the grain produced upon the printing 80 plate is in the form of flakes which are smaller and farther apart at the lighter tones and darker and closer together at the darker tones. This variation in the density 85 of the grain is produced photographically as above described. Also if desired, the sensitizer may be applied separately in the form of a liquid bath in which the plate is immersed after being coated with the other substance above described. This separate 90 application of the sensitizer is especially advantageous when it is desired to keep a number of the coated plates in stock. The plates can thus be kept for a long time without any 95 deterioration and when they are desired for use, the sensitizer may be applied.

Although I have described my improved process in connection with lithography, it will be readily understood that the plate with the novel grain may be used with advantage also in relief and intaglio printing; in certain of the claims, I refer, therefore, to the key plate as the printing plate which may be used outside of the lithographic art. 100

It will thus be seen that I have produced a printing plate which faithfully reproduces photographically every slightest graduation in tone of the original. The record upon this plate is a permanent one, and the 110 ink may be entirely washed away without injuring the printing quality of the plate. The various tones are reproduced through a grain which consists of interwoven sinuous lines or flakes which are lighter and more 115 open at the lighter portions of the picture and heavier and closer together at the darker portions. These relative values of the grain are produced photographically to the finest detail and thus all the very finest 120 graduations in tone are preserved. This makes it possible to obtain true color values with much smaller number of plates than has hitherto been possible. I have found in many cases that three colors, as red, yellow 125 and blue, are sufficient to reproduce all the tints of the original.

My improved process practically elimi-

nates hand work of an artist in the preparation of the lithographic key plate and press plate. All of the corrections necessary may, if desired, be made directly upon the key plate, by closing or opening the grain at the desired point, by the use of a steam or air brush. The use of transfers may be eliminated by using the off-set press to print through the offset roller from the key plate 10 upon the press plate. The latter is etched in a novel manner calculated to prevent injury to the finest detail work.

Although I have described my process in great detail, I desire it to be understood that 15 I do not consider myself limited to these details, as numerous modifications within the spirit of the invention will suggest themselves to those skilled in the art and portions of the improvements may with various degrees of advantage be used without the others.

Having thus described my invention I claim as new and desire to obtain by Letters Patent of the United States:

25 1. A process of preparing a lithographic plate consisting in coating a plate with a gelatinous organic substance, a sensitizing agent capable after exposure to light of rendering such organic substance insoluble in 30 water and an agent which expands upon absorption of moisture and which will not interfere with the sensitiveness of the plate; exposing the plate, washing the same to remove the unexposed portion of the sensitizing 35 agent and then improving the printing quality of the plate by coating the same with a solution of glycerin and sodium chlorid and allowing the same to soak and then heating the same to a temperature considerably below the boiling point.

40 2. A process of preparing a lithographic plate consisting in coating a plate with gelatin, a bichromate and calcium chlorid; exposing the plate, washing the same to remove 45 the unexposed portion of the sensitizing agent and then improving the printing quality of the plate by coating the same with a solution of glycerin and sodium chlorid, and allowing the same to soak and then heating the same to a temperature considerably below the boiling point.

45 3. A process of preparing a lithographic plate consisting in coating a plate with a gelatinous organic substance, a sensitizing agent capable after exposure to light of rendering such organic substance insoluble in water and an agent which expands upon absorption of moisture and which will not interfere with the sensitiveness of the plate; 50 heating the coated plate for a definite period of time corresponding to the grain desired, exposing the plate, washing the same to remove the unexposed portion of the sensitizing agent and then improving the printing quality of the plate by coating the same

with a solution of glycerin and sodium chlorid and allowing the same to soak and then heating the same to a temperature considerably below the boiling point.

55 4. A process of preparing a lithographic plate consisting in coating a plate with gelatin, a bichromate, and an agent which expands upon absorption of moisture and which will not interfere with the sensitiveness of the plate, heating the coated plate 70 for a definite period of time corresponding to the grain desired; exposing the plate, washing the same to remove the unexposed portion of the sensitizing agent and then improving the printing quality of the plate 75 by coating the same with a solution of glycerin and sodium chlorid and allowing the same to soak and then heating the same to a temperature considerably below the boiling point.

80 5. A process of preparing a lithographic plate consisting in coating a plate with gelatin, a bichromate and calcium chlorid, heating the coated plate for a definite period of time corresponding to the grain desired; exposing the plate, washing the same to remove the unexposed portion of the sensitizing agent and then improving the printing quality of the same by coating the same with a solution of glycerin and sodium chlorid and 85 allowing the same to soak and then heating the same to a temperature considerably below the boiling point.

90 6. A process of preparing a lithographic plate consisting in coating a plate with a substratum of sodium silicate dissolved in a solution containing albumen, then adding a coating consisting of a gelatinous organic substance, a sensitizing agent capable after exposure to light of rendering such organic 95 substance insoluble in water and an agent which expands upon absorption of moisture and which will not interfere with the sensitiveness of the plate; exposing the plate, washing the same to remove the unexposed portion of the sensitizing agent and then improving the printing quality of the same by coating the same with a solution of glycerin and sodium chlorid and allowing the same to soak and then heating the same to a temperature considerably below the boiling point.

100 7. A process of preparing a lithographic plate consisting in coating a plate with a substratum of sodium silicate dissolved in a 105 solution containing albumen, then adding a coating consisting of gelatin, a bichromate, and an agent which expands upon absorption of moisture and which will not interfere with the sensitiveness of the plate; exposing the plate, washing the same to remove the unexposed portion of the sensitizing agent and then improving the printing quality of the same by coating the same 110 with a solution of glycerin and sodium chlorid and allowing the same to soak and then heating the same to a temperature considerably below the boiling point.

115 8. A process of preparing a lithographic plate consisting in coating a plate with a substratum of sodium silicate dissolved in a 120 solution containing albumen, then adding a coating consisting of gelatin, a bichromate, and an agent which expands upon absorption of moisture and which will not interfere with the sensitiveness of the plate; exposing the plate, washing the same to remove the unexposed portion of the sensitizing agent and then improving the printing quality of the same by coating the same 125 with a solution of glycerin and sodium chlorid and allowing the same to soak and then heating the same to a temperature considerably below the boiling point.

rid and allowing the same to soak, and then heating the same to a temperature considerably below the boiling point.

8. A process of preparing a lithographic plate consisting in coating a plate with gelatin, a bichromate and calcium chlorid; exposing the plate, washing the same to remove the unexposed portion of the sensitizing agent and then improving the printing quality of the same by coating the same with a solution consisting of one part glycerin in one part of water and a small amount of sodium chlorid according to the humidity of the air, allowing this coating to soak from 15 to 30 minutes, removing the moisture and then drying the plate from two to five minutes at a temperature of about 50° C.

9. A process of preparing a lithographic plate consisting in coating a plate with gelatin, a bichromate, and an agent which expands upon absorption of moisture and which will not interfere with the sensitiveness of the plate, heating the coated plate for a definite period of time corresponding to the grain desired then after exposing the plate, improving the printing quality of the same by coating the same with a solution consisting of one part glycerin in one part of water and a small amount of sodium chlorid according to the humidity of the air, allowing this coating to soak from fifteen to thirty minutes, removing the moisture and then drying the plate from two to five minutes at a temperature of about 50° C.

35 10. A process of preparing a lithographic plate consisting in coating a plate with gelatin, a bichromate and calcium chlorid, heating the coated plate for a definite period of time corresponding to the grain desired; exposing the plate, washing the same to remove the unexposed portion of the sensitizing agent and then improving the printing quality of the same by coating the same with a solution consisting of one part glycerin in one part of water and a small amount of sodium chlorid according to the humidity of the air, allowing this coating to soak from fifteen to thirty minutes, removing the moisture and then drying the plate from two to five minutes at a temperature of about 50° C.

40 11. A process of preparing a lithographic plate consisting in coating a plate with gelatin, a bichromate and calcium chlorid, heating the coated plate for a definite period of time corresponding to the grain desired; then after exposing the plate improving the printing quality of the same by coating the same with a solution consisting of one part glycerin in one part of water and a small amount of sodium chlorid according to the humidity of the air, allowing this coating to soak from fifteen to thirty minutes, removing the moisture and then drying the plate from two to five minutes at a temperature of about 50° C.

12. A process of preparing a lithographic plate consisting in coating a plate with a solution of thirty parts of gelatin to 300 parts of water to which is added 90 parts of a solution of 1 part bichromate, 1 part of calcium chlorid and 10 parts of water, heating a plate so coated at a temperature between 50° and 60° C.; exposing the plate, washing the same to remove the unexposed portion of the sensitizing agent and then improving the printing quality of the same by coating the same with a solution consisting of one part glycerin in one part of water and a small amount of sodium chlorid according to the humidity of the air, allowing this coating to soak from fifteen to thirty minutes, removing the moisture and then drying the plate from two to five minutes at a temperature of about 50° C.

13. A process of preparing a lithographic plate consisting in coating a plate with a gelatinous organic substance, a sensitizing agent capable after exposure to light of rendering such organic substance insoluble in water and an agent which expands upon absorption of moisture and which will not interfere with the sensitiveness of the plate; then printing the image through a usual photographic negative directly upon the plate so coated and washing off the unexposed portion of the sensitizer, said expanding agent serving to break up the coating acted upon by the light into a grain, the density of which corresponds to the degree in which the coating has been acted upon by the light; then weakening or reducing the portions which are too strong by applying warm moisture thereon.

14. A process of preparing a lithographic plate consisting in coating a plate with gelatin, a bichromate and calcium chlorid, then printing the image through a usual photographic negative directly upon the plate so coated and washing off the unexposed portion of the bichromate and gelatin coating, the calcium chlorid serving to break up the coating acted upon by the light into a grain, the density of which corresponds to the degree in which the coating has been acted upon by the light; then weakening or reducing the portions which are too strong by applying warm moisture thereon.

15. A process of preparing a lithographic plate consisting in coating a plate with a gelatinous organic substance, a sensitizing agent, capable after exposure to light of rendering such organic substance insoluble in water and an agent which expands upon absorption of moisture and which will not interfere with the sensitiveness of the plate; then printing the image through a usual photographic negative directly upon the plate so coated and washing off the unexposed portion of the sensitizer and gelatin coating, said expanding agent serving to

break up the coating acted upon by the light into a grain, the density of which corresponds to the degree in which the coating has been acted upon by the light; then reducing portions of the plate which are too strong by spraying steam thereon.

16. A process of preparing a lithographic plate consisting in coating a plate with a gelatinous organic substance, a sensitizing agent capable after exposure to light of rendering such organic substance insoluble in water and an agent which expands upon absorption of moisture and which will not interfere with the sensitiveness of the plate; then printing the image through a usual photographic negative directly upon the plate so coated and washing off the unexposed portion of the sensitizer and gelatin coating, said expanding agent serving to break up the coating acted upon by the light into a grain, the density of which corresponds to the degree in which the coating has been acted upon by the light; then strengthening the portions which are too weak by a blast of air through an air brush with an agent which serves to harden the photographic grain so as to take relatively more ink.

17. A process of preparing a lithographic plate consisting in coating a plate with gelatin, a bichromate, and an agent which expands upon absorption of moisture and which will not interfere with the sensitiveness of the plate; then printing the image through a usual photographic negative directly upon the plate so coated and washing off the unexposed portion of the bichromate and gelatin coating, said expanding agent serving to break up the coating acted upon

by the light into a grain, the density of which corresponds to the degree in which the coating has been acted upon by the light; then strengthening the portions which are too weak by a blast of air through an air brush with an agent which serves to harden the photographic grain so as to take relatively more ink.

18. The process of preparing a printing plate consisting in coating the plate with a printing medium composed of an organic gelatinous substance and a substance capable after exposure to light of rendering such organic substance insoluble in water, heating the plate, then photographically printing the subject thereon, then washing the plate to remove the unexposed sensitized portions thereon and soaking the same in a solution containing a suitable hygroscopic agent.

19. The process of preparing a printing plate consisting in coating the plate with a printing medium composed of an organic gelatinous substance and a substance capable after exposure to light of rendering such organic substance insoluble in water, heating the plate, then photographically printing the subject thereon, then washing the plate to remove the unexposed sensitized portions thereon, soaking the same in a solution containing a suitable hygroscopic agent, then further heating the plate.

Signed at New York in the county of New York and State of New York this 20th day of November, A. D. 1913.

LEO FREUDER.

Witnesses:

Wm. I. COHEN,  
EVE AXEL.